

# United States Patent Office

2,824,798

Patented Feb. 25, 1958

1  
2,824,798

## AUSTENITIC ALLOYS

Wasil W. Dyrcz, Newtonville, Richard K. Pitler, Albany, and Henry M. Butler, Watervliet, N. Y., assignors to Allegheny Ludlum Steel Corporation, Brackenridge, Pa., a corporation of Pennsylvania

No Drawing. Application April 25, 1957  
Serial No. 655,000

5 Claims. (Cl. 75—126)

This invention relates to age hardenable austenitic alloys and, in particular, to age hardenable austenitic alloys which are exceptionally well suited for applications where high levels of strength, ductility and hardness and a moderate degree of oxidation and corrosion resistance are required at temperatures of up to about 1600° F.

In applications such as internal combustion engine exhaust valves and valve components, parts of steam or gas turbines such as wheels, buckets, bolts, combustion liners and tail cone assemblies, the metal industry has made use of alloys containing many different alloying elements and having different mechanical properties. Considerable emphasis has been placed in obtaining alloys which are suitable for use at higher and higher temperatures to increase the efficiency of turbines and the like while at the same time conserving strategic and critical alloying elements. Both price and mechanical properties have been considered in designing the various parts of steam and gas turbines. Most of the foregoing problems have resulted in the selection of alloys having a practical optimum of the foregoing requirements. However, difficulties have been encountered in that a number of these alloys while having the required mechanical properties for use at elevated temperatures prove to be difficult to fabricate or contain high amounts of strategic alloying elements or were exceedingly costly from the standpoint of alloy ingredients and fabrication.

An object of this invention is to provide an age hardenable austenitic alloy having high strength and hardness and which is substantially devoid of strategic, critical or expensive alloying elements.

Another object of this invention is to provide an age hardenable austenitic alloy suitable for use at temperatures of up to 1600° F., said alloy being readily reproducible by standard steel making processes and easily fabricated into the desired components.

A more specific object of this invention is to provide an age hardenable austenitic alloy containing carbon, manganese, silicon, chromium, molybdenum in predetermined amounts and which is devoid of strategic, critical and expensive alloying elements, possesses high strength and hardness and is suitable for use at elevated temperatures of up to 1600° F.

Other objects of this invention will become apparent when read in conjunction with the following description.

This invention in its broadest sense contemplates an alloy comprising from about 0.60% to 1.0% carbon, from about 8.0% to about 15.0% manganese, from about 0.25% to about 1.25% silicon, from about 9.0% to about 15.0% chromium, from about 1.5% to about 4.0% molybdenum and the balance substantially all iron with not more than 1.0% of incidental impurities such as copper, nickel, cobalt, phosphorus, sulfur and other impurities normally found in such alloys. In order to more clearly set forth the composition of the alloy of this invention, reference may be had to Table I illustrating the general range and the preferred range within which the various alloying elements may be varied within the scope of this invention.

2  
Table I.—Composition

| Element | General Range (Percent by Wt.) | Preferred Range (Percent by Wt.) |
|---------|--------------------------------|----------------------------------|
| C       | 0.60-1.0                       | 0.70-0.85                        |
| Mn      | 8.0-15.0                       | 10.0-14.0                        |
| Si      | 0.25-1.25                      | 0.25-1.25                        |
| Cr      | 9.0-15.0                       | 9.0-12.0                         |
| Mo      | 1.5-4.0                        | 2.0-3.5                          |
| Fe      | Bal.                           | Bal.                             |

With respect to the general range of alloying elements set forth hereinabove in Table I, each of the alloying elements in the range given exerts a definite influence on the alloy of this invention. Carbon is necessary for providing sufficient strength and hardness in the alloy and to maintain the alloy substantially austenitic throughout the temperature range of the intended use. Alloys having carbon contents below about 0.60% do not appear to have sufficient strength or hardness whereas alloys with a carbon content in excess of 1.0% while being sufficiently hard have reduced strength and tend to become very difficult to fabricate. Manganese is essential to maintain a stable austenitic structure within the alloy and at least 8.0% manganese is needed. Manganese contents in excess of 15.0% do not appear to substantially contribute to the austenitic stability and have the adverse effect of decreasing the strength of the alloy. Silicon is an essential element and between about 0.25% and 1.25% is necessary. While silicon functions to deoxidize the alloy and contributes to the formation of ferrite, it has only a slight effect upon the rupture strength. Room temperature hardnesses are practically unaffected by variations in silicon content; however, hardnesses when measured at 1400° F. indicate that increasing the silicon content produces a corresponding increase in the hardness. Chromium is a necessary element to provide a sufficient degree of oxidation and corrosion resistance. At least 9.0% chromium is necessary for adequate protection whereas chromium contents in excess of 15.0% have very poor strength characteristics. Chromium has little effect on the hardness of these alloys. Molybdenum is used primarily to increase the strength and hardness of the alloy. At least 1.5% molybdenum is necessary in order to obtain sufficient strength and hardness. Molybdenum contents in excess of 4% while exhibiting sufficient hardness show a decided decrease in the strength such as to detrimentally affect the alloy to an undesirable degree. The balance of the alloy is substantially all iron with incidental impurities.

Within the general range of composition set forth hereinbefore in Table I the test data indicate that there is a preferred range within which the alloying elements may be varied in order to obtain the optimum combination of properties within the alloy of this invention as will be more clearly set forth hereinafter. It has been found that where the carbon content is maintained within the range between 0.70% and 0.85% the optimum combination of strength consistent with good ductility, hardness and austenite stability is obtained. Manganese also exhibits an optimum range in that the optimum combination of strength, hardness, ductility and austenite stability is exhibited where the manganese content is maintained within the range between 10.0% and 14.0%. As was stated hereinbefore silicon is used primarily for deoxidation purposes and its effect upon the alloys of this invention indicates that it is usable throughout the range between 0.25% and 1.25%, there being no optimum range observed. Since chromium is a strong ferritizing element, its use must be limited to provide the optimum

combination between oxidation and corrosion resistance consistent with good ductility, strength and hardness. For this reason it has been observed that chromium contents within the range between 9.0% and 12.0% are quite satisfactory for the purposes of this invention. The preferred range of molybdenum is within the range between 2.0% and 3.5%, it being noted that the optimum combination of strength, hardness and ductility has been observed within the range between 2.0% and 3.5%. This is true as regards the effect of molybdenum on the strength whether the criteria of the time to produce rupture or the time to produce 1% total strain is used as the basis of evaluating the strength.

The alloy of this invention is made in any of the well-known steel making methods, for example, by the carbon-electrode electric arc furnace melting process, the details of which are well known in the art and will therefore not be described. It is sufficient to say that a heat having a composition within the limits set forth hereinbefore in Table I is melted and cast into ingots which can then be readily fabricated into the desired semi-finished mill product by any of the well-known processes, for example, forging, pressing, rolling, extruding and the like. The alloy in the form of a semi-finished mill product may then be fabricated into the desired shape of the finished product and thereafter heat treated as will be more fully described hereinafter, in order to impart optimum mechanical properties thereto. In order to more clearly demonstrate the mechanical properties of the alloy of this invention and the effect of each of the alloying elements upon the mechanical properties, reference may be had to Table II which contains the analysis of a number of heats made and tested, the compositions of which are both within and outside of the scope of the alloy of this invention.

Table II.—Analysis of heats investigated

| Heat  | C    | Mn    | Si   | Cr    | Mo   | Fe   |
|-------|------|-------|------|-------|------|------|
| G-630 | 0.69 | 9.60  | .59  | 11.97 | 1.94 | Bal. |
| G-631 | 0.59 | 9.40  | .59  | 11.93 | 2.04 | Bal. |
| G-632 | 1.10 | 9.43  | .59  | 12.05 | 1.80 | Bal. |
| G-633 | 0.82 | 4.00  | .59  | 12.00 | 2.28 | Bal. |
| G-634 | 0.87 | 6.73  | .56  | 11.81 | 2.10 | Bal. |
| G-635 | 0.90 | 12.64 | .59  | 12.09 | 1.94 | Bal. |
| G-636 | 0.86 | 16.72 | .54  | 11.89 | 2.04 | Bal. |
| G-637 | 0.89 | 10.16 | .28  | 12.01 | 2.00 | Bal. |
| G-638 | 0.80 | 10.49 | .82  | 11.77 | 2.04 | Bal. |
| G-639 | 0.88 | 9.92  | 1.02 | 11.72 | 2.08 | Bal. |
| G-640 | 0.90 | 9.86  | .68  | 8.99  | 2.12 | Bal. |
| G-641 | 0.86 | 9.87  | .52  | 14.90 | 2.05 | Bal. |
| G-642 | 0.86 | 9.80  | .62  | 11.84 | 0.03 | Bal. |
| G-643 | 0.89 | 9.94  | .72  | 11.88 | 3.17 | Bal. |
| G-644 | 0.83 | 9.70  | .50  | 12.13 | 4.78 | Bal. |
| G-688 | 0.85 | 9.59  | .50  | 12.05 | 2.26 | Bal. |

The alloys of Table II were made and tested in order to show the effect of each of the alloying elements on the strength and hardness properties of these alloys. Reference is directed to Table III which contains the results of the tests performed on the alloys of Table II illustrating the effect of a variation of each of the elements of the alloy of the invention on the stress-rupture characteristics thereof. In Table III both the time to rupture and the time to produce 1% total strain are recorded and are used as criteria in evaluating the alloys. The test used to evaluate the stress-rupture properties consisted of subjecting each alloy to a constant load of either 10,000 p. s. i. or 15,000 p. s. i. at a temperature of 1500° F. The time to produce 1% total strain and the time to produce rupture under these conditions of stress and temperature were observed and recorded. Note that all of the alloys were in the heat treated condition when tested. The details of the heat treatment are set forth in Table III.

Table III.—Stress rupture properties

[Test temperature—1500° F. Heat treatment: 2150° F.—1 hr.—W. Q. + 1400° F.—16 hrs.—A. C.]

| Heat No.                       | Stress—15,000 p. s. i. |                             |                  |                        | Stress—10,000 p. s. i. |                             |                  |                        |
|--------------------------------|------------------------|-----------------------------|------------------|------------------------|------------------------|-----------------------------|------------------|------------------------|
|                                | Rupture Time (Hrs.)    | 1% Total Strain Time (Hrs.) | Elong. (Percent) | Red. of Area (Percent) | Rupture Time (Hrs.)    | 1% Total Strain Time (Hrs.) | Elong. (Percent) | Red. of Area (Percent) |
| <b>A. EFFECT OF CARBON</b>     |                        |                             |                  |                        |                        |                             |                  |                        |
| G-631                          | C                      | 305                         | 70               | 13.5                   | 17.8                   | 1,230                       | 490              | 6.8                    |
| G-630                          | .59                    | 610                         | 145              | 10.9                   | 13.1                   | 2,305                       | 760              | 7.0                    |
| G-688                          | .85                    | 463                         | 113              | 10.7                   | 10.4                   | 1,853                       | 345              | 11.2                   |
| G-632                          | 1.10                   | 191                         | 22               | 7.7                    | 11.0                   | .953                        | 145              | 13.7                   |
| <b>B. EFFECT OF MANGANESE</b>  |                        |                             |                  |                        |                        |                             |                  |                        |
| G-633                          | Mn                     | 155                         | 125              | 4.7                    | 3.9                    | 753                         | 465              | 6.0                    |
| G-634                          | 4.0                    | 286                         | 70               | 5.2                    | 3.5                    | 1,236                       | 410              | 6.8                    |
| G-688                          | 6.73                   | 463                         | 113              | 10.7                   | 10.4                   | 1,853                       | 345              | 11.2                   |
| G-635                          | 0.59                   | 463                         | 113              | 10.7                   | 10.4                   | 1,501                       | 390              | 8.0                    |
| G-636                          | 12.64                  | 349                         | 165              | 4.5                    | 9.7                    | 1,501                       | 390              | 4.3                    |
|                                | 16.72                  | 315                         | 97               | 8.0                    | 14.1                   | 1,171                       | 240              | 5.2                    |
| <b>C. EFFECT OF SILICON</b>    |                        |                             |                  |                        |                        |                             |                  |                        |
| G-637                          | Si                     | 403                         | 105              | 12.7                   | 14.1                   | 1,697                       | 500              | 5.7                    |
| G-688                          | .50                    | 463                         | 113              | 10.7                   | 10.4                   | 1,853                       | 345              | 11.2                   |
| G-638                          | .82                    | 217                         | 105              | 3.3                    | 7.8                    | 1,068                       | 235              | 7.7                    |
| G-639                          | 1.02                   | 328                         | 113              | 6.6                    | 6.3                    | 1,678                       | 620              | 9.3                    |
| <b>D. EFFECT OF CHROMIUM</b>   |                        |                             |                  |                        |                        |                             |                  |                        |
| G-640                          | Cr                     | 348                         | 315              | 1.5                    | 3.5                    | 1,186                       | 1,050            | 0.5                    |
| G-688                          | 8.99                   | 463                         | 113              | 10.7                   | 10.4                   | 1,853                       | 345              | 11.2                   |
| G-641                          | 12.05                  | 463                         | 21               | 14.4                   | 27.0                   | .632                        | 305              | 16.6                   |
|                                | 14.90                  | 142                         |                  |                        |                        |                             |                  | 16.0                   |
| <b>E. EFFECT OF MOLYBDENUM</b> |                        |                             |                  |                        |                        |                             |                  |                        |
| G-642                          | Mo                     | 101                         | 16               | 19.4                   | 25.2                   | .484                        | 120              | 11.3                   |
| G-688                          | 2.26                   | 463                         | 113              | 10.7                   | 10.4                   | 1,853                       | 345              | 11.2                   |
| G-643                          | 3.17                   | 394                         | 145              | 6.3                    | 3.5                    | 1,093                       | 360              | 7.4                    |
| G-644                          | 4.78                   | 139                         | 70               | 3.8                    | 2.7                    | 758                         | 330              | 3.8                    |

From the test results recorded in Table III for alloys G-631, G-630, G-688 and G-632 it is seen that in general as the carbon content increases from 0.59% the strength increases to a maximum at about 0.70% to 0.85% carbon and then decreases as the carbon content is further increased to 1.10%. Where the alloys are tested at 1500° F. under an applied stress of 10,000 p. s. i. as well as 15,000 p. s. i. it is found that the optimum strength occurs where the carbon content is in the range between 0.70% and 0.85% as clearly illustrated when both criteria, that is, the time to produce rupture and the time to produce 1% total strain, are compared. The ductility as measured by the elongation and reduction of area is excellent within this range. It will be observed that when the carbon content is increased from about 0.85% for alloy G-688 to about 1.10% for alloy G-632 that there is a definite decrease in the strength of this alloy. It is for this reason that it is preferred to maintain the carbon content at not greater than 1% maximum. Carbon contents below about 0.60% do not appear to have sufficient strength for the purposes of the alloys of this invention. Thus from the considerations of strength and ductility, it is apparent that the alloy of this invention must have a carbon content within the range between 0.60% and 1.0% and preferably within the range between about 0.70% and 0.85% for the optimum in strength and ductility.

The effect of manganese on the alloys of this invention is demonstrated by referring to Subsection B of Table III and the test data recorded therein for alloys G-633, G-634, G-688, G-635 and G-636. It is seen that increasing the manganese content from 4.0% in alloy G-633 to 16.72% in alloy G-636 produces a corresponding increase in both the time to produce rupture and the time to produce 1% total strain when these alloys are tested at 1500° F. and under a stress of 15,000 p. s. i. Thus it is seen that the time to produce rupture is increased from 155 hours for alloy G-633 containing 4.0% manganese, up to a maximum of 463 hours for alloy G-688 containing 9.59% manganese and back to 315 hours for alloy G-638 containing 16.72% manganese. Corresponding behavior is noted when the data of the criteria of 1% total strain is compared. Thus for alloy G-633 having 4.0% manganese it is seen that the time to produce 1% total strain is increased from 125 hours to a maximum of 155 hours for alloy G-688 containing 9.59% manganese. Further increase in the manganese of up to 16.72% for alloy G-636 decreased the time to produce 1% total strain to 97 hours. It is thus apparent that manganese contents in excess of about 15% do not appear to be advantageous to the alloy of this invention. The optimum manganese content is in the range between 10.0% and 14.0% from the standpoint of both strength and ductility. Correspondingly similar results were obtained where the tests were conducted at 1500° F. and under a stress of 10,000 p. s. i. Since manganese does not contribute substantially to the strength of the alloy of this invention but is used predominantly for maintaining a completely austenitic structure, it is sufficient that at least about 8% manganese is used whereas the manganese content should not exceed about 15%. Optimum strength and ductility occur when the manganese content is within the range between 10.0% and 14.0%.

Referring now to Subsection C of Table III and in particular to alloys G-637, G-688, G-638 and G-639, it is seen that increasing the silicon content from 0.28% to 1.02% has little effect upon the rupture strength of these alloys. This is especially borne out by the fact that for the alloys tested at 1500° F., and a stress of 15,000

p. s. i. that the only variation in the time to produce 1% total strain was from 105 to about 113 hours as the silicon content was increased from 0.28% to 1.02%. Since the primary function of silicon is for the purposes of deoxidation and hardness, it is sufficient that the strength is not detrimentally affected throughout the intended range of use. Silicon also contributes to the oxidation resistance of these alloys.

The effect of chromium on the stress rupture properties of these alloys is demonstrated by reference to Subsection D of Table III and in particular to alloys G-640, G-688 and G-641. These data show that chromium contents of 8.99%, 12.05% and 14.9% produce corresponding rupture times of 348, 364 and 142 hours, respectively, when the alloys are tested at 1500° F. and a stress of 15,000 p. s. i. Similar behavior is also noted where the stress is reduced to 10,000 p. s. i. Chromium contents below about 9.0% do not afford a sufficient resistance to oxidation and corrosion for these alloys whereas chromium contents in excess of about 15% detrimentally affect the strength of the alloy so as to make it impractical for use. The optimum combination of strength, ductility, corrosion and oxidation resistance appears to occur where the chromium content is within the range between 9.0% and about 12.0%. This is substantiated where the tests were conducted under a stress of 10,000 p. s. i. as well as 15,000 p. s. i., the temperature in both instances being 1500° F.

Referring now to Subsection E of Table III, the effect of molybdenum is apparent from the test results recorded therein for alloys G-642, G-688, G-643 and G-644. These data illustrate the fact that increasing the molybdenum from about 0.03% up to 4.78% produces a corresponding increase in the time to produce rupture of from 101 hours for alloy G-642 up to a maximum of 463 hours for alloy G-688 and thereafter decreasing such rupture time to 139 hours for alloy G-644, the alloys being tested at 1500° F. and under a stress of 15,000 p. s. i. Similar results were obtained when these alloys were tested at 1500° F. and a stress of 10,000 p. s. i. When the data for the time to produce 1% total strain is examined for the same alloy, it is seen that the maximum time to produce 1% total strain occurs at a somewhat higher molybdenum content than the molybdenum content necessary for maximum time to produce rupture. Thus the maximum rupture life is obtained when the molybdenum content is between about 1.5% and 2.5%, whereas the 1% total strain times are highest for the alloys containing between about 2% and 4% molybdenum. It is thus preferred to maintain the molybdenum content between 2.0% and 3.5% to obtain the optimum combination of strength consistent with good ductility.

From the foregoing, the effect of each of the alloying elements on the stress rupture properties of these alloys is apparent. In all cases, with the exception of silicon, increasing the various alloying elements within the ranges given produces a maximum value of strength which occurs within the preferred range of alloying elements for the alloy of this invention.

The alloys of this invention while having outstanding strength at 1500° F. when tested at stresses of both 10,000 p. s. i. and 15,000 p. s. i., also have excellent hardness properties which make them exceptionally well suited for the uses described hereinbefore. In order to demonstrate these outstanding hardness characteristics, these alloys were tested in both the solution treated and the solution treated and aged conditions, the hardness being measured both at room temperature and at 1400° F. Reference may be had to Table IV which shows the effect of each of the alloying elements on the hardness properties.

7  
Table IV.—Hardness properties

| Heat No.                       | Treatment:<br>2,150° F.—1 Hr.—<br>W. Q. |                    | Treatment:<br>2,150° F.—1 Hr.—<br>W. Q. +1,400° F.—<br>16 Hrs.—A. C. |                    |
|--------------------------------|-----------------------------------------|--------------------|----------------------------------------------------------------------|--------------------|
|                                | Room<br>Temp.<br>(BHN)                  | 1,400° F.<br>(BHN) | Room<br>Temp.<br>(BHN)                                               | 1,400° F.<br>(BHN) |
| <b>A. EFFECT OF CARBON</b>     |                                         |                    |                                                                      |                    |
| G-631                          | .59                                     | 235                | 142                                                                  | 332                |
| G-630                          | .69                                     | 257                | 157                                                                  | 364                |
| G-688                          | .85                                     | 255                | 142                                                                  | 364                |
| G-632                          | 1.10                                    | 282                | 157                                                                  | 418                |
| <b>B. EFFECT OF MANGANESE</b>  |                                         |                    |                                                                      |                    |
| G-633                          | 4.0                                     | 258                | 164                                                                  | 525                |
| G-634                          | 6.73                                    | 262                | 157                                                                  | 503                |
| G-688                          | 9.59                                    | 255                | 142                                                                  | 364                |
| G-635                          | 12.64                                   | 255                | 170                                                                  | 387                |
| G-636                          | 16.72                                   | 260                | 164                                                                  | 375                |
| <b>C. EFFECT OF SILICON</b>    |                                         |                    |                                                                      |                    |
| G-637                          | .28                                     | 255                | 142                                                                  | 375                |
| G-688                          | .50                                     | 255                | 142                                                                  | 364                |
| G-638                          | .82                                     | 255                | 152                                                                  | 364                |
| G-639                          | 1.02                                    | 255                | 164                                                                  | 364                |
| <b>D. EFFECT OF CHROMIUM</b>   |                                         |                    |                                                                      |                    |
| G-640                          | 8.99                                    | 241                | 178                                                                  | 387                |
| G-638                          | 12.05                                   | 255                | 142                                                                  | 364                |
| G-641                          | 14.90                                   | 277                | 157                                                                  | 364                |
| <b>E. EFFECT OF MOLYBDENUM</b> |                                         |                    |                                                                      |                    |
| G-642                          | .03                                     | 241                | 121                                                                  | 332                |
| G-688                          | 2.26                                    | 255                | 142                                                                  | 364                |
| G-643                          | 3.17                                    | 262                | 204                                                                  | 387                |
| G-644                          | 4.78                                    | 269                | 195                                                                  | 387                |

Referring now to alloys G-631, G-630, G-688 and G-632 of Subsection A of Table IV, it is seen that in general the hardness increases as the carbon content is increased from about 0.59% to about 1.10%. Between about 0.7% and about 0.9% there is little difference in the hardness of the alloy in both the solution treated and the solution treated plus aged condition, the hardnesses being measured both at room temperature and at 1400° F. While the values of the hardness are greater where the alloys contain greater than 0.90% carbon, it will be noted as reported in Table III that the strength greatly decreases. Thus the optimum combination of strength, ductility and hardness is exhibited in these alloys when the carbon content is in the range between 0.70% and 0.85%. Alloys with a carbon content below about 0.60% have inferior hardness and strength whereas alloys having a carbon content in excess of 1% have good hardness but poor strength.

Alloys G-633, G-634, G-688, G-635 and G-636 of Subsection B of Table IV illustrate the effect of manganese on the hardness properties. In general, the hardness tends to increase as the manganese content is increased from about 9.0% for alloy G-688 up to about 16.72% for alloy G-636. It will be observed, however, that alloys containing low manganese, that is, alloys G-633 and G-634, exhibit an extremely high room temperature hardness in the solution heat treated and aged conditions. Metallographic examination indicates that the low manganese alloys contain martensite which is a transformation product of unstable austenite. Thus it is clearly established that a minimum of 8% manganese must be maintained within the alloys of this invention in order to maintain a completely austenitic structure. The op-

8  
timum hardness appears to occur between 10.0% and 14.0% which is the same range for optimum strength and ductility as reported in Table III.

The effect of silicon on the hardness of the alloys of this invention is demonstrated by reference to alloys G-637, G-688, G-638 and G-639 in Subsection C of Table IV. As clearly illustrated therein, the room temperature hardnesses of these alloys both in the solution heat treated and the solution heat treated and aged condition are essentially unaffected at room temperature measurements of the hardness where the silicon content is increased between 0.28% to 1.02%. However, when the test results for the hardnesses when measured at 1400° F. are compared both in the solution heat treated and the solution heat treated and aged condition, it is seen that there is a general increase in the hardness as the silicon content is increased from 0.28% to 1.02%. The hardness exhibited throughout the range of silicon tested is sufficiently high that any value in the whole range can be used, there being no optimum range observed.

Referring now to Subsection D of Table IV, the effect of chromium on the hardness properties is clearly demonstrated by reference to alloys G-640, G-688 and G-641. These data show that in general the hardness decreases as the chromium content is increased from 8.99% to 14.90%. The decrease in the hardness observed throughout this range is not appreciable for the alloys in either the solution heat treated or the solution heat treated and aged conditions. The optimum combination of hardness with strength lies in the range between 9.0% and 12.0%.

The most effective element for increasing the hardness is molybdenum. Subsection E of Table IV shows the test results for alloys G-642, G-688, G-643 and G-644 and clearly illustrates that increasing the molybdenum content from 0.03% to 4.78% has produced a corresponding increase in the BHN hardness of from 241 to 269 and from 332 to 387 in the solution heat treated and the solution heat treated and aged conditions, respectively, when measured at room temperature and from 121 to a maximum of 204 and from 137 to 178 in the solution heat treated and the solution heat treated and aged conditions, respectively, when measured at 1400° F. Both the solution heat treated and the solution heat treated and aged hardnesses vary slightly when the molybdenum content is increased from about 3.17% to 4.78%. The optimum combination of properties, that is, strength, ductility and hardness, is obtained where the molybdenum content does not exceed 3.5%.

From the foregoing test data the effect of each of the elements on the hardness of the alloys of this invention is clear. In comparing the strength properties with the hardness properties it is clearly seen that the optimum combination of both strength and hardness occurs when the alloying elements are within the preferred range set forth hereinbefore in Table I. Satisfactory results are also obtained as long as the alloying elements are maintained within the general range as set forth hereinbefore in Table I. However, if the alloying elements are permitted to vary outside of the general range, the strength, ductility or hardness are detrimentally affected so that the alloy is not suitable for its intended use at temperatures of up to 1600° F.

Since the alloy of this invention is completely austenitic it must be hardened by an aging heat treatment in order to obtain the full benefit of its properties. This heat treatment consists of a solution heat treatment at a temperature within the range between about 1950° F. and 2200° F. for a time period of about 1/2 to 8 hours depending upon the section thickness of the alloy or article being heat treated. For most applications the material will be of sufficiently small size so that heating at a temperature of about 2150° F. for about 1 hour will be sufficient to place all of the hardening elements in solution in the alloy. After the alloy is heated for a

sufficient time within the temperature range set forth hereinbefore, it is rapidly cooled by quenching, usually into water. If the size of the article made from the alloy of this invention is sufficiently small in section a less severe quenching medium may be used, for example, air or oil. The solution heat treatment and quenching leaves the alloy article in a soft ductile condition where it can be readily formed and/or machined. The alloy or article is then subjected to an aging treatment at a temperature in the range between 1300° F. and 1600° F. for a time period ranging between 8 and 40 hours depending upon the size. For most applications, an aging time of from 8 to 16 hours will be sufficient. Thereafter, the alloy is air cooled to room temperature. Excellent results have been obtained where the alloy or article made therefrom is solution heat treated at 2150° F. for about 1 hour, water quenched and thereafter aged at a temperature of about 1400° F. for about 16 hours and thereafter air cooled.

The alloy of this invention is especially useful in applications such as valves and valve components. Where the alloy is formed into an article for use in a highly corrosive atmosphere, for example, an exhaust valve or valve component, it may be desirable to provide the article with a protective surface coating to prolong the life of the article. However, where only a moderate corrosive and oxidation environment is encountered, no protective coating is needed or desired.

There are no special skills required in producing, fabricating or heat treating the alloy of this invention. All equipment used is standard and in use in most steel plants today. In particular, the alloy is exceptionally well suited for use at temperatures of up to 1600° F., readily adapts itself to any fabrication operations, is inexpensive from the standpoint of alloying elements used, fabrication procedures employed and heat treatment operations necessary for obtaining optimum properties, and is devoid of strategic, critical and costly alloying elements.

We claim:

1. An austenitic age hardenable alloy suitable for use

20

5 at temperatures of up to 1600° F., consisting of from 0.60% to 1.0% carbon, from 8.0% to 15.0% manganese, from 0.25% to 1.25% silicon, from 9.0% to 15.0% chromium, from 1.5% to 4.0% molybdenum and the balance substantially iron with incidental impurities.

2. An austenitic age hardenable alloy suitable for use

10 at temperatures of up to 1600° F., consisting of from 0.70% to 0.85% carbon, from 10.0% to 14.0% manganese, from 0.25% to 1.25% silicon, from 9.0% to 12.0% chromium, from 2.0% to 3.5% molybdenum and the balance substantially iron with incidental impurities.

15 3. An austenitic age hardenable alloy suitable for use at temperatures of up to 1600° F., consisting of about 0.85% carbon, about 9.59% manganese, about 0.50% silicon, about 12.05% chromium, about 2.26% molybdenum and the balance iron with incidental impurities.

4. As an article of manufacture for use at elevated temperatures of up to 1600° F., an alloy consisting of from 0.60% to 1.0% carbon, from 8.0% to 15.0% manganese, from 0.25% to 1.25% silicon, from 9.0% to 15.0% chromium, from 1.5% to 4.0% molybdenum and the balance iron with incidental impurities, the alloy being formed to the predetermined shape of the article and being in the solution treated condition resulting from quenching the alloy from a temperature in the range between 1900° F. and 2200° F.

25 5. As an article of manufacture for use at elevated temperatures of up to 1600° F., an alloy consisting of from 0.60% to 1.0% carbon, from 8.0% to 15.0% manganese, from 0.25% to 1.25% silicon, from 9.0% to 15.0% chromium, from 1.5% to 4.0% molybdenum and the balance iron with incidental impurities, the alloy being formed to the predetermined shape of the article and being in the age hardened condition resulting from quenching the alloy from a temperature in the range between 1900° F. and 2200° F., and aging the alloy at a temperature in the range between 1300° F. and 1600° F. for a time period ranging between 8 and 40 hours and thereafter air cooling to room temperature.

30

40

No references cited.